

Patented Feb. 4, 1936

2,029,946

# UNITED STATES PATENT OFFICE

2,029,946

## PROCESS OF MAKING PHOTOGRAPHIC EMULSIONS

Max Schmid, Riehen, near Basel, Switzerland,  
assignor to Society of Chemical Industry in  
Basle, Basel, Switzerland

No Drawing. Application December 8, 1933,  
Serial No. 701,531. In Switzerland December  
10, 1932

4 Claims.

(Cl. 95—7)

According to this invention valuable photographic emulsions are obtained by mixing the components necessary for making an emulsion and subsequently ripening the mixture, and, during the ripening stage, withdrawing at least two portions of the emulsion of different degrees of ripening and then uniting these portions.

Emulsions made in this manner have the property that when spread upon a support they give light-sensitive layers which, while of good covering power, have a high sensitivity and a remarkable freedom from halation, even without the usual anti-halation devices. If the emulsion is made from only two withdrawn portions its properties will be influenced according to the degree of ripening of each portion; for instance, if the portion of less ripeness prevails there will be obtained an emulsion which is less sensitive to light and shows steeper gradation and stronger covering power; if the portion of greater ripeness prevails the emulsion will have a high sensitivity and a greater softness.

If the withdrawal of the two portions of different degrees of ripening is carried out by allowing these portions to flow into a common vessel, there is a simplification in the manufacture of the finished emulsion, in that one mixing operation has been unnecessary.

If during the ripening of the emulsion several portions of different degrees of ripeness are withdrawn at short intervals, the emulsion formed by uniting them would have, as compared with one consisting of only two united portions, a better gradation and a greater range of sensitiveness.

By grading the degrees of ripeness of the several withdrawn portions, the properties of the final emulsion may be profoundly influenced; for example, the sensitivity without formation of fog, with retention of covering power, may be still further increased.

As by grading the degree of ripeness of the several portions, whether by raising or lowering the ripening temperature or by prolonging or curtailing the duration of the ripening, or by both these methods, the properties of the emulsion obtained can be profoundly influenced, so also can the properties, particularly the gradation curves, of the finished emulsion be influenced by the ratio in which the portions withdrawn from the ripening mixture are mixed with each other.

For example, if at the beginning of the rise in sensitivity of the ripening there are withdrawn small portions of the emulsion and then the portions afterwards withdrawn continuously in-

creased in quantity, the final emulsion obtained will have softer gradations which, according to the mode of working, will not be at fault or only little so in the shadows. If the quantities of the portions of high degree of ripeness are still further increased at the cost of the quantities of the portions of lower degree of ripeness, one can obtain, with or without the adoption of other conditions which influence the properties of the final product, such as the duration of ripening, ripening temperature, composition of the emulsions or the like, emulsions of which the gradation curves are steeper in the shadows than in the high lights, that is to say, their gamma (angle of the tangent to the curve on the x-axis) is greater in the shadows than in the high lights.

If portions of emulsion are progressively withdrawn during the period of rising sensitiveness to light, final emulsions are obtained which, when brought on to the supports afford extremely valuable photographic layers. These are characterized by high sensitiveness, remarkable durability and high range of sensitiveness with good gradation. The gradations of emulsions obtainable in this manner may be influenced within wide limits by the manufacture of the emulsion and may be adapted to the requirements of the photographic material desired.

As already stated, by varying the stages at which the portions of emulsion are withdrawn from the ripening mass, the properties, for instance general sensitivity, gradation curves, can be influenced almost to any extent in a very simple manner, and this may be assisted by varying other conditions which influence these properties.

Without disadvantageous effect on the emulsions obtained, the increase in sensitivity may be driven by this process up to the beginning of fog.

The present invention may be used for making acid emulsions, ammoniacal emulsions and, if desired, boiled emulsions. By addition of agents which increase sensitivity, the sensitiveness may be further raised, and by the addition of sensitizers color-sensitive layers may be produced.

Accordingly as the emulsions are compounded and accordingly as the ripening is conducted in the present process, layers can be obtained for various purposes of photography and cinematography, for instance, negative films, plates, diapositive layers, reversal films, fine-grain layers, layers sensitive to light for color photography and color cinematography, layers for light-sound production, and developing papers.

These layers serve for making photographic pictures. The negative and positive layers produced by the process may be used alone or in combination with other layers which are obtained from emulsions made by known processes. If as the negative layer there is used one the gamma of which is greater in the shadows than in the high lights, it is particularly advantageous to use as the positive layer one having an analogous gradation curve.

The components necessary for making the emulsion may be mixed at a high or a low temperature. The emulsions which are obtainable in accordance with the invention may be used alone or together with other emulsions made according to this process or to a known process.

The following examples illustrate the invention, the parts being by weight:

*Example 1*

A filtered solution of 1200 parts of silver nitrate, 1100 parts of ammonia (specific gravity 0.91) and 40 parts of citric acid in 6000 parts of water is run, in the course of 20 minutes, into a stirring vessel I containing a solution at a temperature of 28° C. consisting of 6000 parts of water, 600 parts of hard gelatine, 1000 parts of potassium bromide, 20 parts of crystallized sodium carbonate, 18 parts of potassium iodide and 200 parts of an alcoholic solution of erythrosine (1:800). The mixture in this vessel I is now heated gradually to 60° C., while at the same time the mixture is run at an adjustable speed into an additional gelatine solution contained in a stirring vessel II, kept at 25° C. internal temperature, the solution consisting of 2000 parts of water and 300 parts of soft gelatine. In the stirring vessel I the temperature of 60° C. is maintained for about 50-60 minutes and care is taken, by adjusting the speed of outflow, that after this time, according to the desired gradation, all or the greater part of the mixture in vessel I is run into the vessel II cooled to 25° C. When the whole has run out the mixture in vessel II is mixed with a solution of 250 parts of medium- and 250 parts of soft gelatine in 1000 parts of water, the whole is stirred for some time longer and the mixture in vessel II is allowed to solidify by cooling. The completely solid emulsion is cut up into small pieces and in this form thoroughly washed.

Before pouring or spreading this emulsion on the support the pieces are melted together in the stirring vessel I at about 35° C. When the whole has melted to a homogeneous emulsion there are allowed to run, for the purpose of further ripening and if desired with addition of agents that increase sensitiveness, sensitizers or the like, as has been described for the first ripening, portions of the emulsion from the stirring vessel I into a stirring vessel II which contains a solution at 25° C. consisting of 2000 parts of water, 10 parts of potassium bromide, 400 parts of soft gelatine, 300 parts of medium gelatine, 500 parts of alcohol and 100 parts of an aqueous solution of 2 per cent. strength of chrome alum and other additions.

At the beginning of the withdrawal of the emulsion from vessel I into vessel II the temperature in vessel I is raised to 50° C., this temperature is maintained until the desired sensitiveness to light has been attained and all the emulsion is in the vessel II, cooled to 25° C. The filtered emulsion is applied to the supports and dried as usual.

There is obtained an ortho-chromatic photo-

graphic exposure material of high sensitiveness, good covering power and gradation.

By varying the composition of the emulsion by omitting sensitizers or using further sensitizers, and further by varying the ripening process, universal, portrait, dispositive, pan, reversal and other emulsions can be obtained.

*Example 2*

The solutions necessary for making the emulsion are as follows:

|                                                    | Parts |
|----------------------------------------------------|-------|
| Solution I: Water                                  | 6000  |
| Silver nitrate                                     | 1200  |
| Ammonia (specific gravity 0.91) to which are added | 15    |
| Citric acid dissolved in                           | 40    |
| Water                                              | 100   |

|                               | Parts |
|-------------------------------|-------|
| Solution II: Water            | 6000  |
| Hard gelatine                 | 600   |
| Potassium bromide             | 1000  |
| Potassium iodide              | 18    |
| Crystallized sodium carbonate | 20    |
| Erythrosine solution (1:300)  | 25    |
|                               | 300   |

|                     | Parts |
|---------------------|-------|
| Solution III: Water | 3000  |
| Medium gelatine     | 250   |
| Soft gelatine       | 550   |

|                                                    | Parts |
|----------------------------------------------------|-------|
| Solution IV: Water                                 | 2000  |
| Potassium bromide solution of 10 per cent strength | 10    |
| Soft gelatine                                      | 400   |
| Medium gelatine                                    | 300   |

|                                             | Parts |
|---------------------------------------------|-------|
| Solution V: Alcohol                         | 500   |
| Chrome alum solution of 2 per cent strength | 100   |
| Tartrazine solution (1:100)                 | 300   |

Solution I is allowed to flow, while stirring, in the course of 20 minutes into Solution II, kept at 45 a temperature of 28° C. Of the emulsion thus obtained about 6 liters are run into Solution III, kept at 25° C. The temperature of the mixture of Solutions I and II is now raised to 60° C. and is maintained thereat for 30 minutes, when 4 liters of the mixture are run into Solution III, kept at 25° C. The rest of this mixture of Solutions I and II is ripened for a further 50 minutes at 60° C. and is then added to Solution III.

Solutions I, II and III are now mixed. The mixture is allowed to solidify by cooling and the solidified emulsion is washed thoroughly with flowing water.

After the washing and draining the comminuted emulsion (noodles) is melted at 40° C.; of this molten emulsion about 10 liters are run into Solution IV and kept at 30° C., the temperature of the melted noodles is raised to 50-60° C. and kept thereat for about 10 minutes, whereupon 8 liters thereof are run into Solution IV; the residue is further ripened for about 10 minutes at 50-60° C. and also added to Solution IV.

Solutions I, II, III and IV are now mixed together. The mixture is diluted with water to 26 liters and the emulsion allowed to solidify by cooling. The solidified emulsion before it is cast is subdivided into several parts of about the same size as each other. The first part is melted at 50° C., kept at this temperature for 5 minutes and then 75

the second part of the emulsion is added and the procedure continued until all has been melted. To the completely melted emulsion there is then added Solution V and, after mixing, the whole is cooled to about 33° C. and this emulsion is filtered and cast.

If, according to this invention, portions of emulsion are continuously or intermittently withdrawn from the ripening operation in such a manner that at the beginning of the ripening small portions and towards the end of the ripening large portions are withdrawn, highly sensitive ortho-chromatic photographic layers having gradation curves of particular technical value are obtained.

What I claim is:—

1. Process of making photographic silver halide gelatine emulsions by mixing the components necessary for the preparation of the emulsions and ripening the emulsions, consisting in withdrawing during the ripening of the silver halide gelatine emulsion at least two portions thereof, of different degrees of ripeness, and then uniting them.
2. Process of making photographic silver hal-

ide gelatine emulsions by mixing the components necessary for the preparation of the emulsions and ripening the emulsions, consisting in withdrawing during the ripening of the silver halide gelatine emulsion at least two portions thereof, of different degrees of ripeness, into a common vessel.

3. Process of making photographic silver halide gelatine emulsions by mixing the components necessary for the preparation of the emulsions and ripening the emulsions, consisting in withdrawing during the ripening of the silver halide gelatine emulsion several portions thereof, of different degrees of ripeness, into a common vessel, the withdrawal of the several portions being effected at short intervals of time.

4. Process of making photographic silver halide gelatine emulsions by mixing the components necessary for the preparation of the emulsions and ripening the emulsions, consisting in withdrawing during the ripening of the silver halide gelatine emulsion portions thereof, of different degrees of ripeness, into a common vessel, the withdrawal of the portions being continuous.

MAX SCHMID. 25